

1

3,287,266

## LUBRICATING COMPOSITION

Derek Southern, Heswall, Wirral, Francis H. Waight, Little Sutton, Wirral, and Alexander C. B. MacPhail, Eastham, Wirral, England, assignors to Shell Oil Company, New York, N.Y., a corporation of Delaware  
No Drawing. Filed Mar. 30, 1964, Ser. No. 355,949

Claims priority, application Great Britain, Apr. 23, 1963,  
15,953/63

10 Claims. (Cl. 252—46.7)

This invention relates to lubricating oil compositions having improved extreme-pressure properties. In particular, this invention concerns synthetic lubricants containing certain diaryl haloalkyl phosphates.

In recent years, various types of synthetic lubricants have become available to satisfy stringent requirements not met by conventional mineral oils. For example, a major application for synthetic lubricants has been in aircraft turbine engines, which must perform at temperatures as low as  $-65^{\circ}$  F., and maintain stability at temperatures as high as  $400^{\circ}$  to  $500^{\circ}$  F.

One of the most difficult problems encountered in the formulation of synthetic lubricants is imparting extreme-pressure properties to the oil. Various additives have been proposed for making these compositions suitable for lubrication at the high pressures, temperatures, and speeds normally encountered in their use. Although some compounds have successfully contributed good antiwear characteristics, few have also met the equally important requirements of low sludge and deposit formation and thermal stability.

It is an object of the present invention to provide a lubricating composition with excellent extreme-pressure properties which is resistant to sludge and deposit formation and which has good thermal stability.

It has now been discovered that certain diaryl haloalkyl phosphates improve the extreme-pressure properties of lubricating oils to a substantially greater extent than was possible with other known EP agents. Lubricants of the invention contain 0.1 to 10%, preferably 2 to 6% by weight, of a diaryl haloalkyl phosphate of the formula



wherein R is mono- to di-nuclear aryl which is substituted with from 0 to 5, especially 0 to 2 alkyl groups having from 1 to 10 carbons; X is a chalcogen having an atomic number from 8 to 16; R' is non- to di-alkyl methylene wherein alkyl has 1 to 4 carbons; n is an integer from 1 to 6, preferably 1 to 3, especially 1; Y is non- to tri-chloroalkyl having 1 to 2 carbons; and Z is mono- to tri-chloromethyl. Preferred compositions comprise a synthetic base with one or more additives of the invention wherein the above formula one or more of the following is true: R is a phenyl group substituted with from 0 to 2 alkyl groups having 1 to 10 carbons, X is a chalcogen having an atomic number from 8 to 16 (i.e., oxygen or sulfur), R' is methylene, n is 1, Y is non- to tri-chloroalkyl having 1 to 2 carbons (i.e.,  $-\text{CH}_3$ ,  $-\text{CH}_2\text{Cl}$ ,  $-\text{CH}_2\text{Cl}_2$ ,  $-\text{CCl}_3$ ,  $-\text{C}_2\text{H}_5$ ,  $-\text{C}_2\text{H}_4\text{Cl}$ ,  $-\text{C}_2\text{H}_3\text{Cl}_2$ , or  $-\text{C}_2\text{H}_2\text{Cl}_3$ ), and Z is monochloromethyl.

Examples of additives of the invention are phenyl naphthyl 5,5-dichloropentyl 4,4-bis(chloromethyl) phosphate; octylphenyl hexylphenyl 7,7,7-trichloroheptyl 6-chloromethyl 6-dichloromethyl phosphorothionate; (dioctyl) phenyl phenyl 3,3-bis(chloromethyl) 4-chlorobutyl phosphate; dioctylphenyl 2,2-bis(trichloromethyl) 3,3-dichloro-

2

propyl phosphorothionate; diphenyl 3,3-bis(chloromethyl) 4,5-dichloropentyl phosphate.

Particularly preferred diaryl haloalkyl phosphates are diphenyl - 2,2 - bis(chloromethyl) - 3 - chloropropyl phosphate; diphenyl - 2,2 - bis(chloromethyl) - 3-chloropropyl phosphorothionate; dioctylphenyl-2,2-bis(chloromethyl)-3-chloropropyl phosphate; and dioctylphenyl-2,2-bis(chloromethyl)-3-chloropropyl phosphorothionate.

The additives of the invention may be used to impart EP properties to either synthetic or mineral oils, but are preferably used in synthetic ester bases. The ester lubricant bases are preferably aliphatic carboxylic acid esters. These may be esters of a monohydric aliphatic alcohol having from 3 to 18 carbon atoms with a monobasic aliphatic acid having from 4 to 18 carbon atoms, for example, isodecyl pelargonate. A further class of aliphatic carboxylic acid esters which may be used is the aliphatic esters of monobasic carboxylic acids having 4 to 18 carbon atoms and a glycol having 4 to 20 carbon atoms, for example esters of neopentyl glycol, 2-butyl-2-ethyl-propanediol and dipropylene glycol with heptylic acid, n-octoic acid, and pelargonic acid.

A particularly preferred class of aliphatic carboxylic acid esters for use in the lubricating oil compositions of the invention is the aliphatic diester of dibasic carboxylic acids having from 6 to 20 carbon atoms and monohydric alcohols having from 1 to 12 carbon atoms, for example esters of adipic acid, pimelic acid, suberic acid, azelaic acid and sebatic acid with lauryl alcohol, heptyl alcohol, octyl alcohol and nonyl alcohol. Particularly preferred aliphatic diesters of dicarboxylic acids are those derived from monohydric alcohols having a branched chain, for example 2-ethyl hexanol and especially those having no hydrogen on the beta carbon atom, for example 2,2-dimethyl pentanol, 2,2,4-trimethyl pentanol, 2,2,3-trimethyl pentanol, 2,2-dimethylhexanol, and 2-methyl-2-ethyl hexanol.

As examples of other aliphatic carboxylic acid esters which may be used there are mentioned aliphatic esters of monocarboxylic acids having from 3 to 10 carbon atoms, for example, propionic acid, butyric acid, valeric acid, capric acid, caprylic acid, lauric acid and pelargonic acid and polyols, for example, pentaerythritol, dipentaerythritol and trimethylolpropane.

Examples of such esters are pentaerythrityl butyrate, pentaerythrityl tetrabutyrate, pentaerythrityl tetravalerate, pentaerythrityl tetracaproate, pentaerythrityl dibutyratedicaproate, pentaerythrityl butyratecaproate divalerate, pentaerythrityl butyrate trivalerate, pentaerythrityl butyrate tricaproate, pentaerythrityl tributyrat-caproate, mixed  $\text{C}_4\text{--C}_6$  saturated fatty acid esters of pentaerythritol, dipentaerythrityl hexavalerate, dipentaerythrityl hexacaproate, dipentaerythrityl hexahexanoate, dipentaerythrityl hexacaprylate, dipentaerythrityl tributyrat-caproate, dipentaerythrityl trivalerate trinonylate, dipentaerythrityl mixed hexaesters of  $\text{C}_4\text{--C}_{10}$  fatty acids, and trimethylolpropane heptylate.

To illustrate the improved lubricating oil compositions of the present invention the compositions as shown in Table I (Examples IV-VII) were made, tested and compared against the base oil (Example I) and a composition containing the same amounts of a known extreme pressure additive (Examples II and III).

These compositions were tested for their load-carrying capacity on an I.A.E. Gear Rig as described in the Institute of Petroleum Method 166/60T using BSS-EN 34 steel gears and operating at an oil temperature of either  $60^{\circ}$  C. or  $110^{\circ}$  C. The mean failure loads at 2000 r.p.m. and 6000 r.p.m. at both the aforementioned temperatures were determined and recorded in Table II.

TABLE I

| Composition of Example (percent wt.)                           | I     | II   | III  | IV   | V    | IV   | VII  |
|----------------------------------------------------------------|-------|------|------|------|------|------|------|
| Di(isooctyl azelate)                                           | 100.0 | 94.0 | 92.0 | 94.0 | 92.0 | 94.0 | 92.0 |
| Aroclor 1254 (chlorinated diphenyl)                            |       | 3.0  | 5.0  |      |      |      |      |
| Diphenyl-2,2-bis(chloromethyl)-3-chloropropyl phosphate        |       |      |      | 8.0  | 5.0  |      |      |
| Diocetyl phenyl-2,2-bis(chloromethyl)-3-chloropropyl phosphate |       |      |      |      |      | 3.0  | 5.0  |
| 3,7-diocetyl phenothiazine                                     |       | 1.5  | 1.5  | 1.5  | 1.5  | 1.5  | 1.5  |
| Phenyl-alpha-naphthylamine                                     |       | 1.5  | 1.5  | 1.5  | 1.5  | 1.5  | 1.5  |
| 5-methyl benzotriazole, p.p.m.                                 |       | 25   | 25   | 25   | 25   | 25   | 25   |
| Azelaic acid                                                   | 0.02  | 0.02 | 0.02 | 0.02 | 0.02 | 0.02 | 0.02 |
| Silicone MS 200/12,500, p.p.m.                                 | 5     | 5    | 5    | 5    | 5    | 5    | 5    |

TABLE II

| Example                      | I   | II  | III | IV  | V   | VI  | VII |
|------------------------------|-----|-----|-----|-----|-----|-----|-----|
| I.A.E. Scuffing Load (lbs.): |     |     |     |     |     |     |     |
| 2,000 r.p.m.:                |     |     |     |     |     |     |     |
| 60° C.                       | 56  | 83  | 95  | 105 | 130 | 95  | 110 |
| 110° C.                      | 56  | 74  | 80  | 85  | 95  | 85  | 90  |
| 6,000 r.p.m.:                |     |     |     |     |     |     |     |
| 60° C.                       | 34  | 40  | 45  | 50  | 55  | 45  | 55  |
| 110° C.                      | 23  | 32  | 36  | 45  | 50  | 40  | 45  |
| Sum or Scuffing Load (lbs.)  | 169 | 229 | 256 | 285 | 330 | 265 | 300 |

It is apparent from the results in Table II that compositions containing the diaryl haloalkylphosphates of the invention have remarkably superior load-carrying capacities compared to the base stock alone. Indeed, Examples II-VII demonstrate that the EP additives of the invention are considerably more effective than Aroclor 1254, a well-known commercial EP additive.

Diaryl haloalkylphosphates of the invention may be prepared by reacting a haloalkyl oxetane with hydrogen chloride and then treating the alcohol formed with a phosphorochloridate of the formula



wherein R and X are as defined above.

The following preparations are illustrative of the method of preparing the novel phosphates for use as extreme-pressure additives in the compositions of the present invention.

*Preparation I.—Diphenyl-2,2-bis(chloromethyl)-3-chloropropyl phosphate*

3,3-bis(chloromethyl)oxetane (989 g., 6.38 mole) is placed in 2-liter flask fitted with a gas inlet tube reaching to the bottom of the flask, a thermometer and condenser with bubbler tube. The oxetane is heated until molten and then hydrogen chloride is bubbled into the reaction flask for 2 hours during which time the reaction temperature slowly increases to a maximum of 110° C. The product of this reaction is washed with dilute sodium carbonate solution and with water until neutral and then distilled; this product is 2,2-bis(chloromethyl)-3-chloropropanol which gave the following analysis:

Chlorine, percent wt. 53.9 (theory 55.6% wt.).  
Hydroxyl value (meq./g.) 5.12 (theory 5.22).

100 grams (0.52 mole) of 2,2-bis(chloromethyl)-3-chloropropanol, 134 grams (0.5 mole) of diphenyl phosphorochloridate and 50 grams (0.63 mole) of pyridine are placed in a flask and shaken. The mixture temperature slowly rises and thus the reaction flask is water-cooled until the reaction ceases. Toluene (50 ml.) is added and the resulting mixture is refluxed for four hours. When cool, the reaction mixture is further diluted with 50 ml. light petroleum spirit (B.P. 100-120° C.), benzene (50 ml.) and water (50 ml.). The resulting organic layer is washed successively with water, dilute sodium bicarbonate

solution and water until neutral. Water and organic solvent are removed by distillation and the final product is distilled under reduced pressure and on cooling this product crystallizes to a white solid which is diphenyl-2,2-bis(chloromethyl)-3-chloropropyl phosphate and which gave on analysis:

Acid value Nil.  
Free chloride Nil.  
Chlorine (percent wt.) 24.8 (theory 25.1% wt.).

*Preparation II.—Diocetylphenyl-2,2-bis(chloromethyl)-3-chloropropyl phosphate*

Distilled p-octyl phenol (116 g., 0.56 mole) and distilled phosphoryl chloride (43.2 g., 0.28 mole) are placed in a flask fitted with a thermometer and a stirrer. The temperature of the reaction mixture is slowly increased to 228° C. over a period of 2 hours and so maintained for a further 2 hours. The resulting product is distilled through a 12" x 3/4" Vigreux column which is lagged with a heating tape, and the fraction boiling up to 240° C. at 15 mm. Hg pressure analyzed for di-p-octyl phenyl phosphorochloridate. A sample of the phosphorochloridate prepared in this manner gave on analysis: Chlorine (percent wt.), 7.20 (theory 7.20% wt.).

27.6 grams (0.06 mole) of di-p-octylphenyl phosphorochloridate, 13.8 grams (0.07 mole) of 2,2-bis(chloromethyl)-3-chloropropanol as prepared in Preparation I and 6 grams pyridine (0.08 mole) are placed in a flask, the contents shaken and the flask cooled. Toluene is added (50 ml.) and the mixture is refluxed for four hours; two distinct layers are formed in the reaction flask. The product is diluted with 100 ml. of a mixture of light petroleum spirit (B.P. 100-120° C.) and benzene and is then washed with water, dilute sodium bicarbonate solution and water until neutral. The solvent is then distilled. The residue, containing free chloride, is diluted with toluene and the resulting solution is slurried with Amberlite IRA-400 ion exchange resin (activated by washing with NaOH solution). After filtering, the solvent is removed by distillation, leaving an amber-colored liquid product which is di-p-octylphenyl-2,2-bis(chloromethyl)-3-chloropropyl phosphate and which had the following analysis:

Acid value 0.7 mg. KOH/g.  
Free chloride Nil.  
Chlorine (percent wt.) 16.45 (theory 16.42% wt.).

The lubricating oil compositions of the present invention may also contain any of the known additives for

aliphatic carboxylic acid ester lubricating oils, for example, thickeners, antioxidants, anti-lacquering agents, anti-foaming agents, dyes, anti-corrosion agents, metal deactivators and additional extreme-pressure additives if so desired.

Suitable thickeners are polyalkylene glycols and their mono- or di-ethers and esters and the polymers of esters of acrylic or 1-alkyl acrylic acids. Examples of antioxidants which may be used in the lubricating oil compositions according to this invention are alkylated phenols, for example 2,6-ditertiary butyl-4-methyl phenol; alkylated bis phenols, for example, 4,4'-methylene bis(2,6-ditertiary butyl phenol); aromatic amines, e.g., phenyl- $\alpha$ -naphthylamine, phenyl- $\beta$ -naphthylamine, 2,2'-dipyridylamine, diphenylamine and alkyl substituted derivatives thereof. An especially preferred class of antioxidants is the thiiodiarylamines, for example, phenothiazine and 3,7-dioctyl phenothiazine. Mixtures of antioxidants may also be used, particularly mixture containing a thiiodiarylamine, e.g., a mixture of phenothiazine and phenyl- $\alpha$ -naphthylamine.

Suitable anti-forming agents are the polydimethyl siloxanes having viscosities from 100 to 100,000 centistokes at 25° C. Examples of anti-corrosion agents and metal deactivators are benzotriazole, 5-methyl benzotriazole and low molecular weight dicarboxylic acids, e.g., azelaic acid, pimelic acid.

Other extreme-pressure additives which may be used if so desired are, for example, the chloronated di- or polyphenyls and the triaryl esters of phosphorothionic acid.

We claim as our invention:

1. A lubricating oil composition comprising a major proportion of a base lubricating oil and from 0.1 to 10% by weight of a diaryl haloalkyl phosphate of the formula



wherein R is mono- to di-nuclear aryl which is substituted with from 0 to 5 alkyl groups having 1 to 10 carbon atoms; X is a chalcogen having an atomic number of from 8 to 16; R' is non- to di-alkyl methylene, where alkyl has 1 to 4 carbon atoms; n is an integer from 1 to 6; Y is non- to per-chloroalkyl having 1 to 2 carbon atoms; and Z is mono- to tri-chloromethyl.

2. The composition of claim 1 wherein R is phenyl, R' is methylene, and n is 1.

3. The composition of claim 1 wherein X is oxygen.

4. The composition of claim 1 wherein X is sulfur.

5. A lubricating oil composition comprising a major proportion of a synthetic lubricating oil base and from 0.1 to 10% by weight of a diaryl haloalkyl phosphate of the formula



wherein R is mono- to di-nuclear aryl which is substituted with from 0 to 5 alkyl groups having 1 to 10 carbon atoms; X is a chalcogen having an atomic number of from 8 to 16; R' is non- to di-alkyl methylene, where alkyl has 1 to 4 carbon atoms; n is an integer from 1 to 6; Y is non- to per-chloroalkyl having 1 to 2 carbon atoms; and Z is mono- to tri-chloromethyl.

5. The composition of claim 5 wherein the synthetic lubricating oil base is the aliphatic diester of dibasic carboxylic acids having from 6 to 20 carbon atoms and monohydric alcohols having from 1 to 12 carbon atoms.

10 6. A synthetic lubricating oil composition having improved extreme-pressure properties which comprises a major proportion of a synthetic ester base and from 0.1 to 10% by weight of a diaryl haloalkyl phosphate of the formula



20 wherein R is mono- to di-nuclear aryl substituted with from 0 to 2 alkyl groups, alkyl having from 1 to 10 carbon atoms; X is a chalcogen having an atomic number from 8 to 16; Y is non- to per-chloroalkyl having 1 to 2 carbon atoms; and Z is mono- to tri-chloromethyl.

25 7. The composition of claim 7 wherein R is phenyl.

8. A lubricating oil composition comprising a major

30 proportion of a synthetic ester lubricating oil base and from 0.1 to 10% of a diaryl haloalkylphosphate selected from the group consisting of diphenyl-2,2-bis(chloromethyl)-3-chloropropyl phosphate; diphenyl-2,2-bis(chloromethyl)-3-chloropropyl phosphorothionate; dioctyl-35 phenyl-2,2-bis(chloromethyl)-3-chloropropyl phosphate; and dioctylphenyl-2,2-bis(chloromethyl)-3-chloropropyl phosphorothionate.

9. The composition of claim 7 wherein R is phenyl.

35 10. The composition of claim 4 containing an antioxidant selected from the group consisting of 2,6-ditertiary-butyl-4-methyl phenol; 4,4'-methylene bis(2,6-ditertiary-butyl phenol); phenyl-alpha-naphthylamine; phenyl-beta-naphthylamine; 2,2'-dipyridylamine; and diphenylamine.

45

#### References Cited by the Examiner

#### UNITED STATES PATENTS

|           |         |                |          |
|-----------|---------|----------------|----------|
| 2,289,509 | 7/1942  | Malisoff       | 252—49.9 |
| 2,656,373 | 10/1953 | Gamrath        | 260—965  |
| 2,758,091 | 8/1956  | Webber         | 252—49.9 |
| 2,760,937 | 8/1956  | McDermott      | 252—46.7 |
| 3,218,256 | 11/1965 | Edwards et al. | 252—47.5 |

50

55 DANIEL E. WYMAN, Primary Examiner.

L. G. XIARHOS, Assistant Examiner.